

March 3, 1936.

C. P. MARSDEN

2,032,760

CATHODE RAY TUBE

Original Filed June 2, 1933



Charles P. Marsden

INVENTOR

BY *John J. Hogan*

ATTORNEY

## UNITED STATES PATENT OFFICE

2,032,760

## CATHODE RAY TUBE

Charles P. Marsden, Bloomfield, N. J., assignor  
to Hygrade Sylvania Corporation, Salem, Mass.,  
a corporation of Massachusetts

Application June 2, 1933, Serial No. 674,047  
Renewed July 5, 1935

5 Claims. (Cl. 250—27.5)

This invention relates to coating methods and with particularity to coating with fluorescent material.

An object of the invention is to provide a novel 5 method of applying a fluorescent coating to glass or other similar support.

A further object is to provide a novel method of applying a fluorescent coating to a cathode ray tube or similar device.

10 A feature of the invention relates to a cathode ray tube or similar device having a fluorescent coating which has a maximum uniformity.

A further feature relates to the method of attaching the fluorescent coating to the glass or other similar body.

15 Other features and advantages not specifically enumerated will be apparent after a consideration of the following detailed description and appended claims.

20 While the invention finds its greatest practical advantages in the manufacture of so-called cathode ray tubes or Braun tubes, the inventive method is not limited to the manufacture of any particular kind of tube, but is capable of application 25 in any situation where a uniform coating of fluorescent material is to be applied to a supporting member.

In certain types of apparatus, for example cathode ray tubes, Braun tubes, or the like, there 30 is provided a screen which comprises a material that fluoresces or emits light when bombarded by cathode rays or the like. For example, in one known type of construction employed for this purpose, the tube is provided with a constricted 35 or neck portion at one end and an enlarged, substantially flat screen portion at the opposite end, the interior face of this screen portion being provided with this fluorescent coating. Suitable electrodes are provided within the tube for generating, accelerating and oscillating the beam of cathode rays which, upon striking the screen, causes the latter to fluoresce or otherwise emit light rays. Such tubes are customarily used as 40 oscilloscopes for wave analysis, frequency analysis, etc. Tubes of this general type have also been employed for television or picture transmission purposes, in which case the beam or cathode ray not only has its spacial position varied in synchronism with a transmitter, but 45 also the intensity and/or velocity and/or width of the impinging beam are varied to correspondingly vary the intensity of the fluorescent effect from the screen. While, for oscilloscope or similar uses it is important that the fluorescent coating be uniform, minor variations of thickness or

uniformity of the grain in the coating do not seriously affect results. However, in television or similar uses it is absolutely necessary, if truly faithful images are to be reproduced, that the fluorescent coating be not only of the highest uniformity as to thickness, but it is also important that the individual grains constituting the coating be, as far as possible, of the same degree of fineness. It is further highly important in all types of cathode ray tubes that the fluorescent coating be firmly united to the glass or other support, since it is required to be bombarded continuously by the cathode rays.

5 Various methods have heretofore been proposed for applying the fluorescent coating. For example, the most common way is to mix the fluorescent coating with a suitable binder which is then sprayed over the surface to be coated. Needless to say, with ordinary spraying methods it is extremely difficult to secure a coating of uniform thickness. This may be due to a variety of causes. For example, in spraying it is required that the material be sprayed onto the receiving surface at substantially right angles, with the result that if a non-uniform or large grain of 10 material attaches itself to the supporting surface, succeeding traverses of the spray aggravate and accentuate the thickness of the coating at this point. Added to this is the fact that if the coating is not evenly united to the support over its 15 entire surface, the force of the spray may dislodge one or more grains from the coating. Other methods such as painting or the like obviously are incapable of producing uniform coats because of the appreciable physical dimensions of the 20 painting tool as compared with the fine grain 25 constituting the coating.

30 It has been found that a thoroughly uniform fluorescent coating may be achieved in accordance with this invention without spray, painting 35 or similar processes.

In accordance with the invention the surface of the tube to be coated is first provided with a tenuous film of tacky or sticky material or a material which exhibits pronounced adhesive properties for the powdered fluorescent material. This fluorescent material is preferably employed in powdered form and preferably mixed with another powdered weighty material such as powdered zinc or the like. The powdered mixture 45 is then poured or deposited in any familiar manner upon the same film to which it adheres. The support is then rotated, oscillated and/or swirled so as to agitate the powdered mixture relative to the said film, thus distributing the fluorescent 50

powdered material in an even deposit over the film. The excess of powdered material may then be removed by pouring or similar process, after which the support may be heated, baked, or fired to a dull red heat to remove the film and/or binders, resulting in a firm attachment of the fluorescent material onto the glass or other support.

While the foregoing description gives a general plan of the preferred procedure to be employed, a detailed description will now be given of the manner of practicing the invention in connection with a typical form of cathode ray tube.

Referring to the drawing, the numeral 1 indicates generally a glass or other tube having a constricted or neck portion 2 and a flared or enlarged portion 3. The portion 3 terminates in a substantially flat portion 4 which serves to carry the fluorescent material. In accordance with well-known practice in the art of cathode ray tube design, the tube 1 is provided with an emitting cathode represented schematically by the numeral 5, and an electrode or electrodes 6 for varying the intensity of the cathode ray beam. A concentrating or focusing electrode 7 is usually provided to restrict the beam to a comparatively narrow width. A pair of vertical deflecting plates 8 and a pair of horizontal deflecting plates 9 (one shown) are provided for oscillating the cathode ray beam over any predetermined path. A suitable anode or anodes 10 are provided for accelerating the electrons from the cathode 5. The manner of producing and oscillating the cathode ray beam above described constitutes no feature of the present invention and any well-known means may be provided for this purpose.

Prior to attaching the constricted or neck portion 2 to the flared portion 1, the latter flared portion 3 has the interior surface of the wall 4 provided with a tenuous film preferably of the nature of a plasticised lacquer indicated in the drawing by the numeral 11. It is preferred to employ a binder consisting, for example, of a solution of nitro cellulose in a volatile solvent, e. g., ethyl carbonate, amyl acetate, etc. This binder solution is then plasticised preferably by mixing with it 1½% dibutyl phthalate, and in order to retard the drying, a small percentage, such as 1% of diethyl oxalate may be mixed with the binder. It is to be understood, of course, that the invention is not limited to this particular plasticising agent. For example any diamyl or diethyl phthalate or phthalates may be employed or, if desired, dicresyl phosphate may be employed. The invention also contemplates the use of lacquer films containing gums, if these latter gums are burnt out in the final firing. As above stated, the plasticised film is preferably of a tenuous character or sufficiently thin so as to be substantially completely transparent, although it will be understood that any other known transparent film may be employed which, upon firing, is completely removed or becomes transparent.

The film is preferably deposited by pouring or other similar operation. For example, if the portion 4 of the tube is five inches in diameter, approximately 2 cc. of the above material may be dropped on the interior face of the portion 4 and allowed to flow evenly over the surface. Any excess of the material over the required amount may be drained off in any suitable manner, with the result that there is produced a tenuous uniform film which is substantially free from bubbles, flowing marks, etc. This film is then allowed to dry or is dried to the point where it becomes appreciably tacky or sticky, and the excess

of material around the edges may be wiped off or otherwise removed. The drying is then carried slightly further by blowing a gentle current of air into the bulb until the odor of the solvents has substantially entirely disappeared.

After this treatment the film 11 is in a condition such that it will just show finger prints and is now in condition to receive the powdered fluorescent material. Any well-known fluorescent material such as ordinarily employed in cathode ray tubes or the like may be employed. Preferably this material is intimately mixed with a weighty powdered zinc of about 30 mesh. The mixed powdered materials are then poured into the bulb and the bulb is swirled, oscillated, and somewhat violently shaken so as to distribute the relatively fine fluorescent material in an even deposit over the sticky film 11. As a result of this agitating process the heavy grains or particles of zinc or other weighty material cause the powdered fluorescent material to be distributed in a uniform layer over the film 11. One possible explanation for this is that the very fine particles of the fluorescent material are held by a sufficient adhesive force to prevent their dislodgment by the moving or swirling weighty particles of zinc, whereas the non-uniform or enlarged grains of the fluorescent material are carried by the swirling or agitated weighty material, with the result that the fluorescent coat which finally adheres to the film 11 consists of substantially uniform and finely grained fluorescent material. The excess of the powdered materials may then be poured out or otherwise removed from the tube. If, upon examination of the tube it is discovered that there is an excess of fluorescent material forming a lump at any particular portion of the film, this can be removed by adding more zinc or similar weighty material and continuing the swirling action until the lump or non-uniformity is removed. The material having thus been removed, the edges of the coating may be trimmed by rotating the bulb and wiping off the material with a cloth or rubber scraper.

The end 4 of the tube is then subjected to heat preferably to raise it to a dull red heat or to a temperature at which the binder and/or the plasticized film 11 is removed. Preferably also the heat is maintained for a sufficient length of time to bake the fluorescent material onto the member 4.

A tube prepared in accordance with the above coating has been found to possess extremely uniform graining and thickness of fluorescent material and it will be obvious, of course, that various changes and modifications may be made in the described procedure without departing from the spirit and scope of the invention. For example, if desired, the portion 4 of the tube may be slightly heated while pouring in the plasticised lacquer, and this heating may be gradually increased until the film is entirely removed.

If desired, the above procedure may be repeated so as to provide successive coats of fluorescent material, each coating having a thickness practically consisting of a single grain.

The portion 3 thus prepared may then be united or sealed to the neck portion 2 and the tube may then be subjected to the ordinary evacuation and treatment customarily employed in the manufacture of vacuum tube and electron tube devices in general.

What I claim is:

1. A cathode-ray tube having an enclosing en-

velope with a flattened end wall, a cathode, an anode and a deflecting electrode mounted within said envelope, and a coating on the interior surface of said wall consisting of a transparent baked film of a plasticised lacquer carrying a powdery fluorescent material.

2. A cathode-ray tube having an enclosing envelope with a flattened end wall, a cathode, an anode and a deflecting electrode mounted within said envelope, and a coating on the interior surface of said wall consisting of a transparent

baked film of a lacquer containing a phthalate plasticiser and carrying a powdery fluorescent material on its exposed surface.

3. A cathode-ray tube according to claim 2 in which the plasticiser is a diamyl phthalate. 5

4. A cathode-ray tube according to claim 2 in which the plasticiser is a dibutyl phthalate.

5. A cathode-ray tube according to claim 2 in which the plasticiser is dicresyl phosphate.

CHARLES P. MARSDEN. 16